

Patented May 27, 1924.

1,495,614

# UNITED STATES PATENT OFFICE.

JOSEPH SEYER, OF HAWTHORNE, NEW JERSEY, ASSIGNOR TO STANDARD SILK DYEING CO., OF PATERSON, NEW JERSEY, A CORPORATION OF NEW JERSEY.

## PROCESS OF DYEING SILK PIECE GOODS.

No Drawing. Original application filed December 1, 1922, Serial No. 604,390. Divided and this application filed February 24, 1923. Serial No. 621,074.

To all whom it may concern:

Be it known that I, JOSEPH SEYER, a citizen of the United States, a resident of Hawthorne, in the county of Passaic and State of New Jersey, have invented a certain new and useful Process of Dyeing Silk Piece Goods, of which the following is a specification.

This invention relates to a process of dyeing silk, and more particularly to a process 10 of dyeing silk piece goods in certain colors to produce washable silks.

This application is a division of my original application Serial Number 604,390, filed December 1, 1922, Patent No. 1,446,860, and 15 it particularly covers process # 3 described in said original application.

Said process # 3 is applicable for the following colors:

| Chestnut.  | Seal.   | Navy 1.  | Navy 2. | Navy 3.      |
|------------|---------|----------|---------|--------------|
| 20 S. 3925 | S. 3928 | S. 6085  | S. 6925 | S. 6975      |
| Navy 4.    | Brown.  | Tobacco. | Negro.  | Olive brown. |
| S. 6985    | S. 3295 | S. 3945  | S. 3948 | S. 4856      |

The process is conducted as follows: The piece goods are dyed in a continuously boiling water liquor or gum soap liquor, acidulated with (per 250 gallons liquor) 20 lbs. acetic acid, using direct dyes according to the shade desired. They are then treated with about six pounds of tannic acid preferably gradually added to the same gum soap liquor comprising about two hundred fifty gallons of liquor as before at a temperature of 160° F. for one hour. They are then washed well and treated in a cold water bath of two hundred fifty gallons with 4.5 lbs. tartar emetic for 40 minutes, after which they are again well washed. A diazotization is then carried out with 5 lbs. sodium nitrite ( $NaNO_2$ ) in cold water comprising two hundred fifty gallons containing 2 lbs. sulfuric acid per two hundred fifty gallons of liquor. This diazotization, which lasts 20 minutes, is followed by washing well and developing in two hundred fifty gallons of cold water with 45 35 lbs. sodium carbonate ( $Na_2CO_3 \cdot 10H_2O$ ). A cleansing treatment with a soap solution at 160° F. for 40 minutes follows, and the goods are then washed well and acidulated.

In the above-described process direct dyes are mentioned as being suitable for use and in this class may be used pontamine green BBX, diazoline dark brown, accordine seal brown, and others. This list is illustrative, not exhaustive, as other dyes may be used accord-

ing to their nature and shade. The various colors listed may be produced on silk, particularly silk piece goods, by the use of various dyes and combinations of dyes, but for the sake of specific examples the colors listed may

be produced by the use of the following dyes.

Chestnut is obtained by using accordine seal brown, diazoline dark brown, diazoline dark scarlet, and a little chrysophenine G; seal is obtained in the same way plus pontamine green BX; navy 1 is obtained with diazoline sky blue and diazoline dark scarlet; navy 2, 3, and 4 in the same way as navy 1 plus pontamine green BX; brown is obtained with diazoline dark brown, chrysophenine G, pontamine green BX, and diazoline dark scarlet; tobacco, negro, and olive brown in substantially the same way as brown.

As a result of the above process there are produced varieties of dyed silk piece goods which are washable, that is, they may be washed in water containing soap at a tem-

perature of 110° F. and they will, in most cases, stand 180° F. without suffering unevenness in shade or color, or distinct loss of color. In addition to the highly desirable quality of being washable, these piece silks have also the property of being washable without imparting any substantial amount of their color to the washing liquid, such as water or soap solution. My new silk goods have generally the properties described in my aforesaid original application. It is to be understood that where I mention temperatures and other working conditions in an exact and definite manner, I do not limit myself thereto as variations may be made, and I merely mention such conditions in an exact way in order to set forth a preferred embodiment.

While my new silk piece goods have been described as being of unmixed silk, it is also possible to manufacture mixed silk goods, such as silk and cotton, by the above described process, and also other kinds of silk goods.

As many apparently widely different embodiments of my invention may be made without departing from the spirit thereof, I do not intend to limit myself to any particular embodiment except as indicated in the following patent claims.

I claim:

1. The process of treating silk comprising

dyeing it in a continuously boiling liquor with a direct dye, and fixing the dye upon the silk at an elevated temperature.

2. The process of treating silk comprising dyeing it in a continuously boiling liquor with a direct dye and then mordanting the dye with tannic acid at about 160° F.

3. The process of treating silk comprising dyeing it in a continuously boiling acidulated gum soap liquor with a direct dye, adding tannic acid to the same liquor and treating the silk therein at about 160° F.

4. The process of treating silk comprising dyeing it in a continuously boiling liquor with a direct dye, mordanting the dye at a high temperature and diazotizing the dye.

5. The process of treating silk comprising dyeing it in a continuously boiling liquor with a direct dye, mordanting the dye at a high temperature and diazotizing and developing the dye.

6. The process of treating silk comprising dyeing it in a continuously boiling liquor with a direct dye, mordanting the dye at a high temperature, diazotizing and developing the dye and treating with a hot soap solution.

7. The process of treating silk comprising dyeing it in a gum soap liquor containing a direct dye, treating it with tannic acid at 160° F., washing it, treating it with tartar emetic, washing it, diazotizing the dye, washing, developing with sodium carbonate, cleansing with a soap solution, and washing and acidulating.

8. The process of treating silk comprising dyeing it in a continuously boiling liquor with a direct dye, fixing the dye upon the silk at an elevated temperature and treating the silk with a hot soap solution.

9. The process of treating silk piece goods comprising dyeing them in a continuously boiling liquor with a direct dye, and fixing the dye upon the silk at an elevated temperature.

10. The process of treating silk piece goods comprising dyeing them in a continuously boiling liquor with a direct dye and then mordanting the dye with tannic acid at about 160° F.

11. The process of treating silk piece goods comprising dyeing them in a continuously boiling acidulated gum soap liquor

with a direct dye, adding tannic acid to the same liquor and treating the silk therein at about 160° F.

12. The process of treating silk piece goods comprising dyeing them in a continuously boiling liquor with a direct dye, mordanting the dye at a high temperature and diazotizing the dye.

13. The process of treating silk piece goods comprising dyeing them in a continuously boiling liquor with a direct dye, mordanting the dye at a high temperature and diazotizing and developing the dye.

14. The process of treating silk piece goods comprising dyeing them in a continuously boiling liquor with a direct dye, mordanting the dye at a high temperature, diazotizing and developing the dye and treating with a hot soap solution.

15. The process of treating silk piece goods comprising dyeing them in a gum soap liquor containing a direct dye, treating them with tannic acid at 160° F., washing them, treating them with tartar emetic, washing them, diazotizing the dye, washing, developing with sodium carbonate, cleansing with a soap solution and washing and acidulating.

16. The process of treating silk piece goods comprising dyeing them in a continuously boiling liquor with a direct dye, fixing the dye upon the silk at an elevated temperature and treating the silk with a hot soap solution.

17. The process of treating silk piece goods comprising dyeing them in two hundred fifty gallons of a gum soap liquor acidulated with an acid, the dye bath containing a direct dye, treating them in the bath with six pounds of tannic acid at a temperature of 160° F. for one hour, washing them, treating them in a cold water bath of two hundred fifty gallons with four and one-half pounds tartar emetic for forty minutes, washing them, diazotizing the dye, washing, developing with sodium carbonate, cleansing with a soap solution at 160° F. for forty minutes, and washing and acidulating.

In testimony that I claim the foregoing, I have hereunto set my hand this 21st day of February, 1923.

JOSEPH SEYER.